

1

2,893,865

## SINGLE POWDER PHOTOGRAPHIC DEVELOPERS

Laurence G. Welliver and Jerry S. Krizka, Binghamton, N.Y., assignors to General Aniline & Film Corporation, New York, N.Y., a corporation of Delaware

No Drawing. Application December 26, 1956  
Serial No. 630,436

11 Claims. (Cl. 96—66)

The present invention relates to single powder photographic developers in which all of the essential ingredients of the developer are intimately admixed in dry powder form and more particularly, to an improved alkaline stabilizer for such developers.

Photographic developers contain as their essential ingredients one or more organic developing agents such as hydroquinone, 1-phenyl-3-pyrazolidone (phenidone), para-aminophenol hydrochloride, p-methylaminophenol sulfate (metol), pyrogallol, p-phenylene diamine and its N,N-dialkyl substituted derivatives, an alkali such as sodium carbonate, borax, sodium metaborate or the like, a preservative such as an alkali metal sulfite and an anti-foggant such as potassium bromide or sodium bromide. Under ordinary conditions of mixing and storage, such dry developers undergo a decomposition reaction which manifests itself by a color change to a deep brown and adversely affects the photographic activity of the developers. It has always been presumed that this decomposition was caused by the aerial decomposition of the developing agent in the presence of alkali.

The art has been aware of this phenomenon and efforts have been made to abate such decomposition by adding to single powder developer mixtures an acidic stabilizer such as phthalic acid, boric anhydride, metaphoric acid, potassium metabisulfite and the like. While these various acid stabilizers serve to promote the keeping qualities of such developers, they do not lead to optimum results, and developers containing these acidic stabilizers generally discolor within a period of two to three months. Moreover, all of these acidic substances have inherent disadvantages; they are sparingly soluble in water or dissolve very slowly; they react with such components as sulfites and carbonates to form gas which may build up objectionable pressures in sealed cans; their use requires additional alkali in the formula to maintain developer activity; their stabilizing action is seriously impaired when the individual chemicals contain absorbed moisture and/or when the admixture is subjected to humid conditions, and, they provide no noticeable stabilizing action in developers containing alkali metaborates.

It is known that lithium hydroxide has been used in photographic developers as an alkali, particularly for the preparation of highly concentrated liquid developers. When used for this purpose, the lithium hydroxide is employed in combination with other alkali hydroxides to insure that crystallization of developer ingredients does not take place at low temperatures.

We have now discovered that anhydrous lithium hydroxide is an effective stabilizer for single powder photographic developers either alone or in combination with said acid stabilizers. Single powder developers containing anhydrous lithium hydroxide alone or in combination with the usual acidic stabilizers constitute the purposes and objects of the present invention.

The developers which are contemplated herein con-

2

tain, as their essential components, anhydrous lithium hydroxide which serves both as an alkali and a stabilizing agent, an organic developing agent, an alkali, a preservative, an anti-fogging agent, and in most instances, an acid stabilizer. Developers with these components which we have found to be stable during mixing and during storage for considerable periods of time may be compounded in the following proportions, it being understood that all parts are by weight in grams when the resulting dry powder is to be used to make a liter of developing solution:

|                               | Parts     |
|-------------------------------|-----------|
| Lithium hydroxide (anhydrous) | 0.2 to 8  |
| Organic developing agent      | 3 to 15   |
| Alkali                        | 5 to 100  |
| Preservative                  | 30 to 120 |
| Anti-fogging agent            | 0.3 to 2  |
| Acid stabilizer (optional)    | 0.5 to 12 |

The photographic developing agent may be any of those previously mentioned or any of the commonly used developing agents such as pyrocatechol, chlorohydroquinone (adurol), p-hydroxyphenylamino acetic acid (glycin), 2,4-diaminophenol (amidol). These developing agents may be used alone or in admixture with each other. Typically, we may use a mixture of metol and hydroquinone, metol and 1-phenyl-3-pyrazolidone (phenidone), phenidone and hydroquinone or phenidone, metol and hydroquinone.

The preservative is an alkali metal sulfite preferably sodium sulfite usually in its anhydrous condition, the antifogging agent is sodium or potassium bromide or one of the organic anti-fogging agents such as 6-nitrobenzimidazole, 5-nitrobenzimidazole, 2-mercaptopbenzimidazole, 5-chlorobenzimidazole, 6-chlorobenzimidazole, tetrazole or benzotriazole. The alkali may be any of those used in compounding photographic developers, such as sodium carbonate, potassium carbonate, borax (sodium tetraborate), sodium metaborate, disodium phosphate, or the like. If desired, larger amounts of sodium sulfite can be used without the need for additional alkali, in which cases the sodium sulfite acts both as an alkali and a preservative.

Among the acidic stabilizers which can be used are not only those enumerated above but also maleic anhydride, phthalic anhydride, benzoic anhydride, salicylic acid, phthalimide, saccharin, and anhydrous oxalic acid.

In compounding the aforesaid developer mixtures, one may proceed by first mixing the acidic stabilizer or stabilizers, adding and admixing the alkali, then the developing agent and finally the other ingredients, adding the anhydrous lithium hydroxide last. However, if it be preferred, all the ingredients may be admixed simultaneously.

The use of anhydrous lithium hydroxide offers many advantages and represents a marked improvement over the previously used stabilizers. The fact that lithium hydroxide is a strong alkali makes it possible to substitute all or part of the alkali normally used in a developer with a weaker alkali. For example, it is possible to use borax instead of sodium metaborate, bicarbonate instead of carbonate, and to use sodium sulfite without sodium carbonate. Moreover, single powder developers containing the usual acidic stabilizers absent the anhydrous lithium hydroxide discolor in a period of a few months. When, however, the acidic stabilizers and the anhydrous lithium hydroxide are present together in a single powder developer, the stability of the developer is greatly magnified and no discoloration appears even after storing the developer for more than 12 months.

One of the most important advantages of anhydrous lithium hydroxide lies in the fact that its stabilizing action

is not impaired to the extent of other known stabilizers when the chemicals are subjected to humid conditions such as during storage and blending. In this connection, it is noteworthy that anhydrous lithium hydroxide may be combined with sodium bisulfite or potassium metabisulfite to provide a truly superior stabilizing action. This is surprising in view of the fact that sodium bisulfite or potassium metabisulfite exert only a mild stabilizing action which is practically non-existent under humid conditions. Yet, it reinforces very markedly the much better stabilizing action of lithium hydroxide. Somewhat similar results are obtained by combining lithium hydroxide with such acidic stabilizers as phthalic acid and saccharin.

It is manifest, the facts being as stated, that the results must be attributable to some peculiar coaction between the anhydrous lithium hydroxide and the acidic stabilizer which serves to greatly intensify the stabilizing action of the acidic component, particularly of the alkali bisulfites and metabisulfites.

The following examples will serve to illustrate our invention but are not restricted thereto. The quantity of the single powder developers represented by the following formulae is to be dissolved in sufficient water to give one liter of developer solution and the components are blended as previously indicated.

#### Example I

|                                | Gm.  |
|--------------------------------|------|
| p-Methylaminophenol sulfate    | 0.75 |
| Sodium sulfite (anhydrous)     | 11   |
| Hydroquinone                   | 3    |
| Sodium carbonate (monohydrate) | 16   |
| Potassium bromide              | 0.5  |
| Lithium hydroxide (anhydrous)  | 1.2  |

This paper developer which is free from acidic stabilizers kept for 6 months without discoloration or decomposition.

#### Example II

|                               | Gm. |
|-------------------------------|-----|
| Metol                         | 1.5 |
| Sodium sulfite (anhydrous)    | 80  |
| Hydroquinone                  | 3   |
| Borax                         | 3   |
| Potassium bromide             | 0.5 |
| Lithium hydroxide (anhydrous) | 1.2 |
| Potassium metabisulfite       | 6.4 |

This borax containing fine-grain developer remained stable without discoloration for more than a year.

#### Example III

|                               | Gm. |
|-------------------------------|-----|
| Metol                         | 1.5 |
| Sodium sulfite (anhydrous)    | 80  |
| Hydroquinone                  | 3   |
| Borax                         | 3   |
| Potassium bromide             | 0.5 |
| Lithium hydroxide (anhydrous) | 0.3 |
| Potassium metabisulfite       | 1.6 |

This developer which contained lesser amounts of lithium hydroxide and potassium metabisulfite than the developer of Example II, did not show any discoloration after 6 months storage.

#### Example IV

|                            | Gm.  |
|----------------------------|------|
| Metol                      | 1.5  |
| Sodium sulfite (anhydrous) | 80   |
| Hydroquinone               | 3    |
| Boric acid                 | 1.9  |
| Potassium bromide          | 0.5  |
| Lithium hydroxide          | 0.35 |

This fine-grain developer which contained only lithium hydroxide as a stabilizer remained stable for more than 6 months.

#### Example V

|                                | Gm. |
|--------------------------------|-----|
| p-Methylaminophenol sulfate    | 4   |
| Hydroquinone                   | 10  |
| 5 Sodium sulfite (anhydrous)   | 45  |
| Sodium carbonate (monohydrate) | 64  |
| Potassium bromide              | 0.9 |
| Lithium hydroxide (anhydrous)  | 0.9 |
| Phthalic acid                  | 0.6 |
| 10 Potassium metabisulfite     | 1.5 |

This paper developer did not decolorize or show any other signs of decomposition when stored for more than a year.

#### Example VI

|                                   | Gm.  |
|-----------------------------------|------|
| Metol                             | 1.3  |
| Hydroquinone                      | 3.7  |
| Sodium sulfite (anhydrous)        | 12.8 |
| 20 Sodium carbonate (monohydrate) | 24   |
| Potassium bromide                 | 0.5  |
| Lithium hydroxide (anhydrous)     | 0.8  |
| Potassium metabisulfite           | 4    |

This energetic single-powder negative developer kept without decomposition or discoloration for more than a year.

#### Example VII

|                                 | Gm.  |
|---------------------------------|------|
| Ethylenediamine tetracetic acid | 0.8  |
| 30 Phenidone                    | 0.4  |
| Hydroquinone                    | 10   |
| Phthalic acid                   | 0.75 |
| Potassium metabisulfite         | 2    |
| 35 Sodium sulfite (anhydrous)   | 40   |
| Sodium carbonate                | 30   |
| Potassium bromide               | 3.8  |
| Lithium hydroxide (anhydrous)   | 3    |
| Benzotriazole                   | 50   |

40 This X-ray type single powder developer could be stored without decomposition for more than a year.

#### Example VIII

|                                 | Gm.  |
|---------------------------------|------|
| Ethylenediamine tetracetic acid | 0.8  |
| 45 Potassium metabisulfite      | 2    |
| Phthalic acid                   | 0.5  |
| Phenidone                       | 0.5  |
| Hydroquinone                    | 9    |
| 50 Sodium sulfite (anhydrous)   | 67.5 |
| Sodium carbonate (monohydrate)  | 45   |
| Potassium bromide               | 2    |
| Lithium hydroxide (anhydrous)   | 1.5  |
| Potassium iodide                | 20   |

55 This single powder developer which serves as a first developer for color film of the reversal type could be stored for more than a year without decomposition or discoloration. If desired, an alkali thiocyanate on the order of (2-3 grams) sodium thiocyanate per liter may be added as a silver halide solvent.

Modifications of the invention will occur to persons skilled in the art. We, therefore, do not intend to be limited in the patent granted except as necessitated by the appended claims.

We claim:

1. A stable single powder photographic developer containing, an organic silver halide developing agent, an alkali, a preservative, an anti-fogging agent and a stabilizing amount of anhydrous lithium hydroxide.
2. The composition as defined in claim 1, wherein said stabilizing amount is on the order of from 0.2 to 8 grams based on the amount of developer powder required to make up one liter of developer solution.
3. A stable single powder photographic developer containing a mixture of an organic silver halide developing

75

agent, anhydrous lithium hydroxide, an alkali metal salt of sulfurous acid and an anti-fogging agent.

4. A stable single powder photographic developer containing in addition to an organic silver halide developing agent, an alkali, an alkali metal salt of sulfurous acid, an acidic stabilizing agent selected from the group consisting of boric anhydride, metaboric acid, phthalic anhydride, phthalic acid, salicylic acid, phthalimide, saccharin, maleic anhydride and anhydrous oxalic acid and an anti-foggant; a stabilizing amount of anhydrous lithium hydroxide.

5. A stable single powder photographic developer containing as its essential components for the preparation of a liter of developing solution:

|                                                                                                                                                                                                                                                                 | Grams       | 15 |
|-----------------------------------------------------------------------------------------------------------------------------------------------------------------------------------------------------------------------------------------------------------------|-------------|----|
| Lithium hydroxide (anhydrous)                                                                                                                                                                                                                                   | 0.2 to 8    |    |
| Organic silver halide developing agent                                                                                                                                                                                                                          | 3 to 15     |    |
| Alkali                                                                                                                                                                                                                                                          | 5 to 100    |    |
| Alkali metal sulfite                                                                                                                                                                                                                                            | 30.0 to 120 |    |
| Anti-fogging agent                                                                                                                                                                                                                                              | 0.3 to 12   | 20 |
| And an acid stabilizer selected from the group consisting of alkali bisulfites, alkali metal bisulfites, boric anhydride, metaboric acid, phthalic anhydride, phthalic acid, salicylic acid, phthalimide, saccharin, maleic anhydride and anhydrous oxalic acid | 0.5 to 12   |    |

6. A stable single powder developer composition containing a mixture comprising anhydrous lithium hydroxide, an organic silver halide developing agent, an alkali selected from the group consisting of alkali borates, alkali sulfites and alkali carbonates, and an acidic stabilizer selected from the group consisting of alkali bisulfites, alkali metabisulfites, boric anhydride, metaboric acid, phthalic anhydride, phthalic acid, salicylic acid, phthalimide, saccharin, maleic anhydride and anhydrous oxalic acid.

7. A stable single powder developer having the following composition:

|                               | Grams | 40 |
|-------------------------------|-------|----|
| p-Methylaminophenol sulfate   | 1.5   |    |
| Sodium sulfite (anhydrous)    | 80    |    |
| Hydroquinone                  | 3     |    |
| Borax                         | 3     |    |
| Potassium bromide             | 0.5   |    |
| Lithium hydroxide (anhydrous) | 1.2   | 45 |
| Potassium metabisulfite       | 6.4   |    |

8. A stable single powder developer having the following composition:

|                               | Grams |
|-------------------------------|-------|
| p-Methylaminophenol sulfate   | 1.5   |
| Sodium sulfite (anhydrous)    | 80    |
| Hydroquinone                  | 3     |
| Borax                         | 3     |
| Potassium bromide             | 0.5   |
| Lithium hydroxide (anhydrous) | 0.3   |
| Potassium metabisulfite       | 1.6   |

9. A stable single powder developer having the following composition:

|                               | Grams |
|-------------------------------|-------|
| p-Methylaminophenol sulfate   | 1.5   |
| Sodium sulfite (anhydrous)    | 80    |
| Hydroquinone                  | 3     |
| Boric acid                    | 1.9   |
| Potassium bromide             | 0.5   |
| Lithium hydroxide (anhydrous) | 0.35  |

10. A stable single powder developer having the following composition:

|                                | Grams |
|--------------------------------|-------|
| p-Methylaminophenol sulfate    | 4     |
| Hydroquinone                   | 10    |
| Sodium sulfite (anhydrous)     | 45    |
| Sodium carbonate (monohydrate) | 64    |
| Potassium bromide              | 0.9   |
| Lithium hydroxide (anhydrous)  | 0.9   |
| Phthalic acid                  | 0.6   |
| Potassium metabisulfite        | 1.5   |

11. A stable single powder developer having the following composition:

|                                | Grams |
|--------------------------------|-------|
| p-Methylaminophenol sulfate    | 1.3   |
| Hydroquinone                   | 3.7   |
| Sodium sulfite (anhydrous)     | 12.8  |
| Sodium carbonate (monohydrate) | 24    |
| Potassium bromide              | 0.5   |
| Lithium hydroxide (anhydrous)  | 0.8   |
| Potassium metabisulfite        | 4     |

#### References Cited in the file of this patent

#### UNITED STATES PATENTS

2,739,894 Rasch et al. Mar. 27, 1956

#### OTHER REFERENCES

Handbook of Chemistry and Physics, 38th ed. (1956-57), page 540.